

# UNITED STATES PATENT OFFICE.

OTTO EISENSCHIML, OF CHICAGO, ILLINOIS, ASSIGNOR, BY MESNE ASSIGNMENTS, TO  
NEW PROCESS FILLER CO., OF CHICAGO, ILLINOIS, A CORPORATION OF ILLINOIS.

## SHOE-FILLING COMPOSITION.

1,224,153.

Specification of Letters Patent.

Patented May 1, 1917.

No Drawing.

Application filed June 16, 1915. Serial No. 34,416.

*To all whom it may concern:*

Be it known that I, OTTO EISENSCHIML, a citizen of the United States, residing in the city of Chicago, county of Cook, and 5 State of Illinois, have invented certain new and useful Improvements in Shoe-Filling Compositions, of which the following is a specification.

In manufacturing welted shoes, before applying the outer sole to the bottom of the shoe, it is necessary to fill up the cavity in the under side of the insole in order to prepare a level foundation for the outer sole. a number of different compounds have been 15 developed for this purpose, the manner of applying these compounds being substantially as follows:

The compound, after first being heated to a temperature considerably higher than 20 maximum ordinary atmospheric temperatures, is taken up in small quantities by the operator, by means of a spoon or spatula, and placed in the cavity, the mass being afterward, while still warm and plastic, 25 squeezed level into the interstices of the shoe cavity by means of considerable pressure exerted through a heated roll or other device.

However, so far as I am aware, a filler 30 which is absolutely satisfactory in every respect has heretofore not been produced. Some of these filler compounds are not completely plastic when heated to a working temperature, or cannot be spread evenly 35 with a knife; for this reason excessive pressure must be employed in order to squeeze the material evenly into all parts of the cavity, which necessitates the provision of more or less complicated machinery for applying the compound to the shoe. Some of 40 these compounds have a very disagreeable, penetrating odor, which frequently becomes quite pronounced when the shoe is worn in hot weather, or in any place where the shoes 45 may happen to be stored or kept.

Other fillers are not sufficiently sticky when applied and do not adhere properly to the leather on either side of the filler, which seriously affects the wearing quality of the 50 shoe, in that this defect frequently causes the filler to bunch up, roll, or travel under the movement of the foot and cause the formation of high spots on the sole which results in undue wear at these points.

55 The essential features of a shoe-filling

compound are, first, cohesiveness; second, adhesiveness; and third, a proper melting point. The composition must be sufficiently adhesive to stick to the surfaces of the inner and outer soles; it must have the proper 60 amount of coherency so that it will not disintegrate, crack or crumble, while at the same time, its melting point must be higher than the maximum atmospheric temperature, and, on the other hand, low enough to prevent 65 damage to the leather during its application to the shoe. In the effort to obtain all of these desirable features, the binder has heretofore been composed of a number of different substances or ingredients of widely different physical and chemical 70 properties; for instance, such substances as dextrin, wax tailings, rosin, and lubricating oil have been used in the same compound. Naturally, such a composition is 75 quite expensive to manufacture and is in the nature of a compromise. In such a compound, the ingredients are not chemically combined with each other, but are simply 80 mixed together mechanically, the mixture thus having no inherent chemical stability whatever.

A shoe-filler compound should be absolutely waterproof at all times so that if water, by any chance, does leak through the 85 outer sole, it will be arrested by the filler and prevented from penetrating to the interior of the shoe. However, it has been found that in attempting to make fillers which will answer all other requirements, 90 the waterproofing qualities of the compound have been considerably sacrificed. Some of these compositions, although waterproof when applied to the shoe and for a short time afterward, gradually lose their waterproofing qualities. Many fillers are tempered with oil in order to reduce the melting point, and this oil, in most cases, gradually separates out of the compound in course of time, being absorbed by the leather; this separating out of the oil from the compound, in addition to impairing the waterproof qualities of the shoe, has the effect of hardening the compound and of thus 105 making the sole of the shoe comparatively inflexible and uncomfortable for the wearer. In some cases the pliability of the filler is so impaired by this process that its original flexibility almost disappears and the bending of the shoe causes the mass of filler 110

to crack and disintegrate. The hardening of the compound, with the resulting inflexibility of the sole, often ruins the shoe in a comparatively short time, this hardening effect being particularly pronounced where rosin is used as one of the ingredients, since this substance becomes very brittle in cold weather.

The object of my invention is to provide a compound for filling shoes which will be entirely free from the above enumerated defects or disadvantages in use, and which will possess other meritorious qualifications, as will hereinafter appear.

At the present time the tendency is to make shoes as light as possible, consistent with proper wearing qualities. The wearer insists that a modern shoe should be of extremely light weight and yet have as long or a longer life than the old-fashioned heavy-weight shoe; and to this end, I select as the body of my improved filler a material which has a very low specific gravity. An excellent material for this purpose is cork, which, besides having a low specific gravity, possesses a high degree of resiliency, which it retains practically indefinitely.

The body material for which, as stated, I prefer cork, is comminuted by shredding finely or by granulating into particles considerably larger than the grains of ordinary coarse white sugar. It is then ready for incorporating with the binder; that is, the material which is used to bind the individual particles of the filler-body together into a coherent mass, and at the same time impart to the compound the necessary waterproof and other properties.

After discarding a vast number of different materials, as a result of numerous experiments extending over a long period of time, I have discovered that prepared asphaltum possesses all of the physical and chemical properties which are required in a perfect binder. The term "asphaltum," as loosely employed, includes a large number of mineral compounds which, although mainly hydro-carbon in character and having substantially the same chemical composition, possess widely differing physical properties. This is especially true of the melting point, which varies greatly, depending upon the degree of refinement and the process employed in preparing the asphaltum for the market. Although the chemical composition of the various asphaltic compounds varies slightly, I have found that many asphaltums are suitable for my purpose, provided that they have a melting point of approximately 120° F., which is high enough to prevent the compound from liquefying or becoming fluid at ordinary atmospheric temperatures, while at the same time it is unnecessary to heat the compound

to a dangerous or excessive temperature when applying the filler to the shoe. The melting point of the asphaltum is not sharply defined, the fusing of the mass being gradually effected as the temperature is raised from 110° F. to 130° F.

No particular skill or special apparatus is required for mixing together the binder and the body material. In practice, I heat the asphaltum under a slow fire in a caldron or kettle. After the mixture has attained the required degree of uniformity and fluidity, the cork is added and thoroughly stirred and mixed, the mixture being meanwhile maintained at a sufficient temperature to prevent solidifying of the binder. Enough body material is added to the liquid binder to thoroughly coat the particles and cause them to adhere together and prevent the presence of voids in the finished filler compound. I find that this requires about one part of comminuted body material, by weight, to three parts, by weight, of the asphaltic binder. Such a combination results in the formation of a substantially homogeneous mass, practically free from voids, while at the same time it has the right degree of plasticity when heated to a working temperature.

One of the particular benefits or advantages derived from the use of my compound for filling shoes is due to the fact that no particular skill or special machinery or apparatus is necessary in order to apply the compound to the shoe. This is due to the fact that asphalt, when heated to the fusing point, does not become instantly fluid but remains in a semi-plastic condition, with a somewhat buttery consistency, over a comparatively wide range of temperature around the fusing point. While in this condition, it does not stick to hot metal, and thus the compound can be spread in the shoe cavity with the same ease as butter upon bread. After having heated the compound to a temperature of approximately 160° F., the workman, by means of a spoon or dipper, places in the shoe cavity the required quantity of heated filler compound, and afterward, by means of a hot spatula or spreader knife, is enabled to evenly and uniformly spread the compound in the cavity. The free working qualities of the material when hot are such that only a comparatively slight amount of pressure on the knife or spatula is required in order to force the compound into the corners or interstices of the shoe cavity. Thus I obviate the necessity of supplying expensive and cumbersome steam-heated rolls or other apparatus for applying pressure to the filler compound after it is applied to the shoe, although such apparatus may be used wherever already installed.

After the shoes have been filled, it is

unnecessary to store them in a drying room or to let them stand for any considerable length of time, since the mixture sets practically instantaneously, or, at any rate, as soon as the temperature reaches that of the ordinary atmosphere. I thus save the expense of providing sufficient space to store the shoes while the filler body is curing or setting, and I also save the loss due to the 10 delay in the cycle of manufacturing operations.

After numerous practical experiments which I have conducted with my improved filler, I find the compound is very flexible 15 under all conditions, it does not age or lose its resiliency in course of time, and it will not check, crack, or disintegrate after years of service in a shoe. It is absolutely unaffected by atmospheric conditions, retaining 20 its original elastic and waterproof properties in hot, cold, wet, or dry climates.

It has been found in many cases that the soles of shoes which were filled with all of the filler compounds which have so far been 25 brought to my attention were completely spoiled if the shoes were allowed to remain at a high temperature for a considerable time; for instance, if placed on the top of a steam radiator and allowed to remain there 30 over night. This latter practice, by the way, although a most reprehensible one, is not so uncommon as might be imagined. The reason that such heating spoiled the shoes was because of the fact that in those 35 old filler compounds, the application of considerable heat for a sustained period causes the binder of the filler compound to split up or separate out into its various ingredients, the binders, as heretofore stated, not being 40 homogeneous chemical substances, but merely mechanical mixtures of such incongruous materials as dextrin, rosin and oil. The result was that the oil oozed out and the 45 filler was ruined. The great advantage of asphaltum in this respect is, first, the fact that it is a homogeneous chemical unit, and, second, that its viscosity, even at high temperatures, is very high so that it does not easily penetrate the pores of leather or other 50 small crevices. Long continued tests by heating shoes filled with my improved compound to a sustained temperature of 150° F. indicate that no separation whatever takes place between the cork and the asphaltum 55 binder, which is a single, homogeneous, chemical compound and contains no ingredient which might have a tendency to separate out or be absorbed by the leather.

My improved filler has a natural adhesive- 60 ness which makes it stick tightly to the inner and the outer sole, and prevents the compound from balling up, rolling, or traveling in bunches under the action of walking while the shoe is warm. The layer of filler 65 thus retains its original thickness in the

cavity between the inner and the outer soles and causes the shoe to retain its shape, and consequently lengthens its life considerably. There is no oozing of the binder through the 70 leather or the seams or interstices of the shoe, and a shoe filled with compound is absolutely free from objectionable smell or odor, owing to the fact that the binder does not contain volatile ingredients which dry out or evaporate from the binder after the 75 shoe is produced.

The compound is absolutely waterproof under all conditions and after years of service, the waterproof quality of the shoe being greatly enhanced by the natural adhesiveness of the compound, which causes it to stick tightly to the sides of the cavity and prevents gaps or channels which would admit moisture to the interior of the shoe. The compound is particularly resilient or 80 flexible and retains its pliability indefinitely, so that a shoe filled with my improved compound is originally very flexible and comfortable to wear and does not stiffen up in 85 course of time.

In the course of my experiments I have discovered that asphaltum differs widely from the substances which have heretofore been used in shoe filler compounds, in that it is possible to add to the asphaltum quite a 90 considerable percentage of certain oils, for instance, a fairly heavy mineral lubricating oil, without sacrificing the inherent chemical stability of the material, which has previously been referred to. This feature is of 95 some importance when it is desired to obtain a rather more fluid binder in case the asphaltum has a somewhat higher melting point than is required. The chemical affinity between the asphaltum and the oil which is 100 added thereto for tempering, is so great and the asphaltum is of such viscosity, that even where the quantity of oil added to the binder is as high as ten or fifteen per cent., there is 105 absolutely no tendency for the oil to separate out from the compound even if the latter be heated to a high temperature for a long period of time.

One of the most important advantages of 110 my invention is due to the relative cheapness of the asphalt compound, which can be purchased in the open market for a very few cents per pound. This enables me to manufacture my shoe-filler vastly cheaper than many of the old compounds containing 115 a long list of comparatively expensive ingredients which must be prepared or compounded at high cost by skilled labor. In addition to the cheapness of my compound, which costs much less per pound than the 120 shoe-filler compounds which have heretofore been brought to my notice, I have found that it will fill more shoes of a standard size than will the old materials; for instance, one pound of any of the standard filler com- 125

pounds heretofore in use will fill approximately forty pairs of shoes, whereas my material will run about fifty pairs to the pound.

Although I have described what I consider to be a preferred embodiment of my invention, it should be understood that the details of the composition may be varied somewhat without departing from the spirit of the invention, which I do not wish to limit, except as specified in the appended claims.

I claim—

1. A shoe-filler compound, composed of a

body of comminuted cork and a binder of mineral asphaltum having a melting point of approximately 120° F.

2. A shoe-filler compound having the following composition: one part, by weight, of comminuted cork, and three parts, by weight of a mineral asphaltum having a melting point of approximately 120° F.

OTTO EISENSCHIML.

Witnesses:

C. A. SOANS,  
EMILIE ROSE.